

# United States Patent

Kowalski

[15] 3,706,635

[45] Dec. 19, 1972

[54] **ELECTROCHEMICAL COMPOSITIONS  
AND PROCESSES**

[72] Inventor: Xavier Kowalski, St. Louis, Mo.

[73] Assignee: Monsanto Company, St. Louis, Mo.

[22] Filed: Nov. 15, 1971

[21] Appl. No.: 199,036

[52] U.S. Cl. .... 204/46, 204/43, 204/44,  
204/45 R, 204/48, 204/49, 204/50 R, 204/52

R, 204/54 R, 204/55 R, 204/DIG. 2

[51] Int. Cl. .... C23b 5/02, C23b 5/46

[58] Field of Search .. 204/45 R, 46, 47, 48, 49, 50 R,  
204/50 Y, 51, 52 R, 52 Y, 53, 54 R, 54 L, 55  
R, 55 Y, 43, 44, DIG. 2; 106/1; 117/130 E

[56] **References Cited**

## UNITED STATES PATENTS

3,475,293 10/1969 Haynes et al..... 204/48

3,617,343 11/1971 Kandler et al..... 106/1 X

## FOREIGN PATENTS OR APPLICATIONS

1,539,226 9/1968 France ..... 204/46

1,909,144 9/1970 Germany ..... 204/46

2,023,304 11/1970 Germany ..... 204/45

Primary Examiner—G. L. Kaplan  
Attorney—James J. Mullen et al.

[57] **ABSTRACT**

An electrically conductive medium for the electrodeposition of metals is described which comprises an aqueous solution of a composition comprising (1) a complex consisting of a metal ion and an ethylenediamine tetra(methylene phosphonate) ligand, and (2) a complex consisting of a metal ion and a 1-hydroxy, ethylidene-1,1-diphosphonate liquid.

**9 Claims, No Drawings**

## ELECTROCHEMICAL COMPOSITIONS AND PROCESSES

The present invention relates to the electrodeposition or electroplating of metals and to novel media which may be employed in the electrodeposition or electroplating of metals. The invention further relates to novel processes for the preparation of such media and to novel processes for the electrodeposition of metals.

Processes for the electrodeposition of metals are well known and involve electrolyzing an electrically conductive medium (e.g., an electroplating bath — also known as a galvanic solution) which usually comprises an aqueous solution of an inorganic metal cyanide. The metal of the metal salt dissolved in such a medium is usually the metal which it is desired to electrically deposit upon a substrate.

Classically the electrodeposition or electroplating system consists of an electroplating bath and two or more electrodes in which the cathode or cathodes comprise the object upon which the metal is to be deposited. The anode usually, although not necessarily, consists of a solid metal or metal alloy containing metal identical to the metal of the plating metal ions in the electroplating bath. Such metal ions will be transformed into a film or plate of elemental metal as they are electrically deposited upon the cathode.

Electroplating baths (galvanic solutions) are usually aqueous alkaline solutions or dispersions of metal cyanides and often have disadvantages (depending upon the particular metal ion and/or the particular surface on which the metal ion is to be deposited) of producing relatively dull or lusterless plates or coatings and/or deposits of coatings of uneven thickness. Furthermore, the use of metal cyanide solutions can be hazardous since, if the pH of the electroplating medium should drop to neutral or below, there is a danger of poisonous hydrogen cyanide gas being produced. Also the use of metal cyanides presents a disposal problem due to their toxicity and such disposal, unless the cyanides are dumped into sewers or streams in which they cause pollution, is expensive.

It has been proposed heretofore in U.S. Pat. No. 2,195,409 to partially overcome some of the disadvantages of dull plates or plates of uneven thickness by adding to an electric bath, containing a metal cyanide, a nuclear alkyl derivative of an aromatic sulfonic acid of the benzene series (as distinguished from nuclear alkyl derivatives of condensed polynuclear aromatic sulfonic acids such as those of the naphthalene series). According to this patent the presence of a small amount of an alkyl aromatic sulfonate eliminates pitting (e.g., uneven thickness) and the formation of pin holes in the metal plate. Further according to this patent the plates are bright, uniform deposits of metal. Still further, according to this patent, employment of such sulfonates has a further advantage in that they act as emulsifying agents and also form soluble salts with many of the metals used in electroplating. However, these organic compounds are used with metal cyanides and the resulting media possess the disadvantages possessed by metal cyanides.

Basically, the problems connected with the cyanide electroplating were overcome as pointed out in the inventions described and claimed in U.S. Pat. No. 3,475,293 via the utilization of certain diphosphonates

or mono-amino lower alkyl phosphonates. As a supplement and improvement to the inventions of U.S. Pat. No. 3,475,293, I have now found that certain "compositions" comprising two different species of organophosphorus compounds are cooperatively effective in electroplating plating baths over an extensive pH range and said baths are characterized by having a high degree of stability over a wide temperature range.

In accordance with the present invention, it has been found possible to electrically deposit certain hereinafter defined metals on a wide variety of substrates or basis metals by the use of certain aqueous solutions or dispersions of hereinafter defined complexes of metal ions and two different species of organophosphorus compound ligands. The electrolysis of these solutions or dispersions (having an extensive pH range) results in metal deposits of uniform thickness which have a continuity and a brightness which can be controlled as desired.

It is one object of this invention to provide a novel electrically conductive medium which may be employed in the electrodeposition of metals.

It is a further object of this invention to provide processes for preparing an electrically conductive medium.

It is a still further object of this invention to provide processes for electroplating or electrically depositing a wide variety of metals on a spectrum of substrates.

Still further objects of the present invention will become apparent from the following description and the appended claims.

The present invention provides, in part, an electrically conductive medium comprising an aqueous solution (or dispersion) of a composition comprising (1) a complex consisting of a metal ion and an ethylenediamine tetra(methylene phosphonate) ligand of the formula:



wherein M is hydrogen, alkali metal (such as sodium, potassium, lithium and the like) ammonium, alkylammonium and amine; and (2) a complex consisting of a metal ion and a 1-hydroxy, ethylidene-1,1-diphosphonate ligand of the formula:



wherein M is the same as described above. The "two complex"-containing composition is present in such solution (or dispersion) in an amount sufficient to electrically deposit the metal of a metal ion when an electric current is passed through said solution (or dispersion). More specifically, it is found that the use of this "two complex"-containing composition results in a unique cooperative effect as contrasted to the use of either complex "(1)" or "(2)" above on an individual

basis. This cooperative effect is quite unexpected as will be seen from the results hereinafter described in the Examples.

It is to be understood that the following terms, phrases or words used hereinafter, have the meanings so indicated:

- a. "aqueous solution" - includes and means both a solution and a dispersion of the "composition" (described below).
- b. (aqueous solution of a) "composition" - includes and means both of the complexes "(1)" and "(2)" described above, and/or a single complex consisting of a metal ion, the ethylenediamine tetra(methylene phosphonate) ligand, and the 1-hydroxy, ethylidene-1,1-diphosphonate ligand.
- c. "EDTMP" or "ethylenediamine tetra(methylene phosphonate) ligand" - includes and means all of the compounds falling within Formula I above (e.g., full acid, salts and partial salts).
- d. "HEDP" or "1-hydroxy, ethylidene-1,1-diphosphonate ligand" - includes and means all of the compounds falling within Formula II above (e.g., full acid, salts and partial salts).

Regarding items (c) and (d) above, it is to be understood that where one so desires, and there is no substantial adverse effect on the desired end result, an ester (full or partial) of EDTMP and/or HEDP could be employed.

In the above medium (galvanic bath), the metal ion is advantageously a metal ion from the group cobalt, silver, tin, gold, copper, iron, nickel, zinc and cadmium ions. The particular metal employed to form the aforementioned complexes with the EDTMP and HEDP ligands will generally depend upon the metal which it is desired to electrically deposit.

It is to be understood that the metal ions to be employed are preferably those water-soluble metal compounds which form chelates with EDTMP and HEDP, i.e., the chelate constituents. Illustrative, but not limiting, metal compounds used in the present invention can be (1) simple ionic metal salts which, when dissolved, set free a metal ion capable of a chelate formation, for example, copper sulfate, or (2) they are more complex salts which, when dissolved, give a metal ion capable of a chelate formation, for example, sodium zincate, or (3) metal salts, such as the carbonates, which react with the EDTMP and HEDP chelate constituents, and form metal chelate salts. Furthermore, the plating of alloys can be accomplished according to the invention by the use of two or more different metals capable of a chelate formation used in correct proportions. As examples of the plated alloys of the invention, there may be mentioned copper-nickel alloys and copper-zinc alloys "yellow brass" and "white brass."

The amounts of metal ions (in the form, for example, of water-soluble metal salts) and the EDTMP and HEDP ligands utilized in the electroplating medium or galvanic baths can vary depending upon several variables such as bath temperature, pH, substrates to be plated, water-solubility of the "composition," i.e., the metal ion - EDTMP and HEDP complexes, and the like. Of the above-described composition, it is preferred to be water soluble to an extent such as to provide from about 0.1 percent to about 5 percent by weight, preferably 1 percent to about 5 percent by

weight, based on the total weight of said aqueous solution, of a transitional metal ion (in water when dissolved therein). However, suitable electroplating baths of the invention can also be prepared by using from about 0.01 to about 400 grams of the EDTMP-HEDP (chelate constituent) per liter; a concentration of 50 to 150 grams per liter is utilized effectively.

Within the "composition" per se, it is a critical feature of this invention that the mole ratios of EDTMP and HEDP to metal ion be within a certain range in order to produce the cooperative effect heretofore described. Regarding HEDP, the mole ratio of HEDP to metal ion is from about 1:1 to about 4:1, preferably from about 1.5:1 to about 3:1. Regarding EDTMP, the mole ratio of EDTMP to metal ion is from about 0.1:1 to about 1:1, preferably from about 0.25:1 to about 1:1. In all cases, however, it is critical that the mole ratio of HEDP to metal ion be higher in numerical value than the mole ratio of EDTMP to metal ion. For example, where the mole ratio of HEDP to  $Cu^{++}$  is 1:1, the mole ratio of EDTMP to  $Cu^{++}$  must be less than 1:1, such as 0.9:1. Additionally, where the mole ratio of HEDP to  $Cu^{++}$  is 4:1, the mole ratio of EDTMP to  $Cu^{++}$  can be as high as 1:1.

It is to be understood that outside of the foregoing molar ratios, the cooperative effect does not manifest itself. For example, in the electrodeposition of copper, it has been found in the present invention experimentation that increasing the amount of EDTMP ligand (above that stated above) in the overall "composition" narrows the "brightness range" (hereinafter defined) by producing wider "burns" in the high current density area. Conversely, decreasing the amount of EDTMP ligand (above that stated above) in the overall "composition" results in a less effective plating in a low current density area or in a lower "covering power."

The amount of the "composition" comprising a metal ion and the EDTMP-HEDP ligands which may be present in the electrically conductive medium may vary considerably and will usually depend upon the solubility of the "composition." Generally speaking, the amount of "composition" is based upon the amount of metal employed and the "composition" is usually present in an amount which is sufficient to provide from about 0.1 percent to about 5 percent by weight, based on the weight of the aqueous solution of metal in the form of metal ion. Such "compositions" comprising these metal complexes are usually substantially soluble under these circumstances. The particular concentration of the "composition" within the above range will depend primarily upon the particular metal of the metal complexes. Thus, for example, when a divalent metal ion is iron or copper, the concentration of the "composition" preferably is a concentration sufficient to provide from about 1 percent to about 5 percent by weight of copper or iron. When the metal of the metal complexes is nickel, the concentration of the "composition" is preferably a concentration sufficient to provide from about 1.5 to about 3 percent by weight of the nickel. In the case of zinc the concentration of the "composition" is preferably such as to provide a concentration from about 2 percent to about 5 percent by weight of the zinc; and in the case of cadmium the concentration of the "composition" is preferably such as to provide a concentration from about 1 to about 4 percent by weight of cadmium.

As noted hereinbefore the electrically conductive medium, which comprises an aqueous solution of the "composition" comprising the metal complexes, has a wide pH range, for example, a pH range of from about 6.0 to about 13.0; however, lower and higher pH's are operative. The pH of the medium will depend to some extent upon the metal ion of the metal complexes, the alkali metal or hydrogen cation and also to some extent upon the substrate upon which the metal ion is to be electrically deposited in the elemental state. Thus, by way of example, when the electrically conductive medium comprises an aqueous solution of divalent copper and the EDTMP—HEDP ligands, the pH of the medium may be in the range of from about 6.0 to about 13.0, the higher pH's being attained when M in the above described Formulas I or II is an alkali metal cation instead of a hydrogen cation. If the electrically conductive medium containing a copper complex is to be used, for example, in plating copper on steel or brass, the pH of the medium is preferably in the range of from about 7.0 to about 10.5. If the electrically conductive medium containing copper EDTMP-HEDP complexes is to be used for plating, for example, copper on aluminum the pH of the medium may be in the range of from about 7.0 to about 12.

If the electrically conductive medium comprises an aqueous solution containing iron ions and the EDTMP—HEDP ligands, the medium preferably has a pH in the range of from about 7.0 to about 10.0. When such medium is to be used, for example, to deposit iron on brass the pH of the medium preferably is in the range of from about 6.0 to about 11.0, whereas if the medium is to be used, for example, to deposit iron on zinc the pH of the medium preferably should be in the range of from about 7 to about 10.

When the electrically conductive medium comprises an aqueous solution of a complex containing nickel ions and the EDTMP—HEDP ligands, the pH of the medium preferably should be in the range of from about 6.5 to about 11. Media having pH's within this range have been found to be particularly advantageous when it is desired to deposit nickel on zinc, brass or steel.

When the electrically conductive medium comprises an aqueous alkaline solution of a composition containing divalent zinc ions and the EDTMP-HEDP ligands, the pH of the medium usually should be in the range of from about 6.5 to about 12, preferably in the range of from about 7.5 to about 10, and such a medium has been found particularly advantageous in the electrodeposition of zinc on steel and brass. When the electrically conductive medium comprises an aqueous alkaline solution of a composition containing divalent cadmium ions and the EDTMP—HEDP ligands, the pH of such medium usually should be in the range of from about 7.0 to about 11.0, preferably in the range of from about 8.0 to about 10.0, and such medium has been found to be particularly advantageous in the electrodeposition of cadmium on steel or brass.

The electrically conductive medium, comprising the aqueous solution of the "composition," may be prepared in a variety of ways which will depend upon the particular class or species of the individual ligands which it is desired to employ to form the metal complexes and more particularly the metal (ion) which it is desired to complex with the ligands. Although in many

instances the metal complexes may be synthesized prior to its dissolution or dispersion in water, it has been found generally desirable to dissolve component precursors of the complexes in water to form the composition containing the desired metal ion and the EDTMP—HEDP ligands. The components of the composition which usually comprises the EDTMP—HEDP ligands, an alkali metal ion and a divalent metal ion, may be dissolved in the aqueous medium (usually water) simultaneously or in any order. However, it has been found advantageous and preferred to dissolve the EDTMP—HEDP ligands in water containing the alkali metal and thereafter to add the metal, usually in the form of a water soluble metal salt, to the medium.

It has been found particularly advantageous to disperse the EDTMP-HEDP ligands either in the acid form or in the alkali metal "ester" form and to add to the resulting solution the metal (ion), in the form of a water soluble salt consisting of the metal (ion) and a nonoxidizing anion. Alternatively, the EDTMP—HEDP ligands, in the acid form, may be dissolved in water, the metal (ion) salt added to the solution and thereafter the alkali metal is dissolved in the solution. The anions of the metal salts, e.g., the metal (ion) and the alkali metal salts, are preferably nonoxidizing anions such as, for example, sulfate, chloride, phosphate, citrate, carbonate, oxide, or acetate anions. For example, anions such as carbonate or sulfate anions are preferred for copper cations.

When the EDTMP—HEDP ligands are added as the hydrogen or acid form, it may also be desirable to add the alkali metal, in the form of a water soluble alkali metal salt, containing any of the anions referred to above. When it is desired, for example, to prepare an aqueous alkaline dispersion of a "composition" comprising divalent copper ions and the EDTMP—HEDP ligands either in the acid or alkali metal form appropriate quantities of copper carbonate, the EDTMP—HEDP ligands in the acid form, and an alkali metal carbonate are dissolved in water with agitation. During the addition of the ingredients, when a carbonate is employed, carbon dioxide is evolved and the resulting dispersion is free of the added anions thus eliminating the necessity for pH adjustment due to the presence of the anion. By so proceeding, as will be evident hereinafter from the Examples, there is provided an aqueous alkaline solution of a "composition" from which, when an electric current is passed therethrough, the metal (ion) can be deposited upon a suitable cathode.

A plating bath which has been found particularly advantageous may be prepared by first dissolving the full acids of EDTMP and HEDP in water. To the resulting solution there is added the desired amount of metal salt and the resulting solution may then be adjusted to the desired pH by the addition of an alkali metal carbonate.

The present invention further provides a process for the electrodeposition of a metal (ion) which comprises the steps of electrolyzing an aqueous solution of a "composition" comprising metal complexes consisting of any of the metal ions hereinbefore described and the EDTMP—HEDP ligands. The amount of "composition" present in the solution is, for example, an amount sufficient to provide from about 1 percent to about 5 percent by weight, based on the weight of the disper-

sion, of said metal. By so proceeding, metals such as copper, iron, nickel, zinc and cadmium may be electrically deposited on a cathode comprising substrates such as steel, aluminum, brass, zinc and the like.

During the electrolysis, that is, the passing of an electric current through the aqueous solution, the bath is maintained at a temperature of from just above the freezing point to just below the boiling point of the aqueous solution, generally from room temperature to 90°C. For reasons of current efficiencies, it has been found preferable to maintain the temperature of the electrically conductive medium in the range of from about 40°C to about 80°C.

The amount of current employed in the electrodeposition may vary widely depending upon the particular metal ion in the form of complexes with the EDTMP—HEDP ligands, the particular EDTMP—HEDP ligands, the temperature of the medium and whether or not the medium is agitated during the passage of the electric current therethrough. Generally, the amount of current employed will be a current sufficient to provide a current density of from about 0.5 to about 300 amperes per square foot of electrode surface. Ordinarily when the current is passed through an electrically conductive medium which is quiescent or unagitated, the current employed will be an amount sufficient to provide a current density of from about 1 to about 150 amperes per square foot and when the electrically conductive medium is agitated the current employed will be an amount sufficient to provide a current density in the range of from about 1 to about 300 amperes per square foot of electrode surface. The amount of current employed will depend to some extent on the metal (ion) which it is desired to deposit.

When it is desired, for example, to deposit or to electroplate copper, the electrically conductive medium will comprise an aqueous alkaline solution containing complexes of divalent copper ions and the EDTMP—HEDP ligands and the current employed will be preferably an amount sufficient to provide a current density of from about 1 to about 120 amperes per square foot of electrode surface. When such electrically conductive medium is not agitated the preferred amount of current will be an amount preferably sufficient to provide a current density in the range of from about 2 to about 60 amperes per square foot. When the medium is agitated the amount of current employed will be an amount sufficient to provide the current density of from about 2 to about 120 amperes per square foot.

In preferred processes, when it is desired to electrodeposit copper, the electrically conductive medium (the galvanic or plating bath) will comprise an aqueous alkaline solution containing divalent copper ions and EDTMP—HEDP ligands. The current employed preferably is an amount sufficient to provide a current density of from about 1 to about 100 amperes per square foot of electrode surface. When the medium is not agitated the preferred amount of current will be an amount sufficient to provide a current density in the range of from about 2 to about 50 amperes per square foot of electrode, whereas when the medium is agitated, the preferred amount of current employed will be an amount sufficient to provide a current density of from about 10 to about 100 amperes per square foot of electrode.

When it is desired to deposit or electroplate nickel, the electrically conductive medium will comprise an aqueous alkaline solution containing divalent nickel ions and EDTMP—HEDP ligands, and the current employed will usually be an amount sufficient to provide a current density of from about 1 to about 300 amperes per square foot of electrode surface.

When such electrically conductive medium is unagitated the amount of current will be that which 10 preferably will provide a current density in the range of from about 5 to about 150 amperes per square foot, whereas when the medium is agitated the amount of current will preferably be an amount sufficient to provide a current density of from about 2 to about 50 amperes per square foot of electrode surface.

When it is desired to electrodeposit zinc, the electrically conductive medium will comprise an aqueous alkaline solution containing complexes of divalent zinc ions and EDTMP—HEDP ligands, and the current employed will be an amount sufficient to provide a current density of from about 1 to about 50 amperes per square foot of electrode surface. When the medium is not agitated, the preferred amount of current employed will be an amount sufficient to provide a current density of from about 1 to about 25 amperes per square foot whereas, when the medium is agitated, the current employed will be an amount sufficient to provide a current density of from about 1 to about 50 amperes per square foot of electrode surface.

When it is desired to electrodeposit cadmium, the electrically conductive medium will comprise an aqueous alkaline solution containing complexes of divalent cadmium ions and EDTMP—HEDP ligands. The current employed will be an amount sufficient to provide a current density of from about 1 to about 50 amperes per square foot of electrode surface. When the electrically conductive medium is not agitated the preferred amount of current will preferably be an amount sufficient to provide a current density in the range of from about 2 to about 40 amperes per square foot whereas if the electrically conductive medium is agitated, the amount of current will preferably be an amount sufficient to provide a current density of from about 1 to about 50 amperes per square foot of electrode surface.

The time required to electroplate or to electrically deposit the metals will vary with the current density in the medium and will depend upon the thickness of the plate or deposit which it is desired to obtain. Generally, the greater the current density, the shorter will be the time required to produce a deposit or plate comprising a given thickness of electrically deposited metal.

In accordance with a preferred embodiment of the processes of this invention, it has been found possible to electrically deposit copper on a wide variety of basis metals or substrates such as zinc, iron, brass, steel, aluminum and the like. This preferred process comprises passing an electric current, at a density in the range of from about 5 to about 150 amperes per square foot of electrode surface, through an aqueous alkaline solution containing complexes of divalent copper ions and potassium salts of the EDTMP—HEDP ligands, i.e., hexapotassium ethylenediamine tetra(methylene phosphonate) and tetrapotassium 1-hydroxy, ethylenediamine-1,1-diphosphonate, having a pH in the range of from about 7.0 to about 10.0. The amount or concentration of the composition containing these complexes

in the solution is an amount sufficient to provide from about 1 percent to about 5 percent by weight, based on the weight of the solution, of copper and the temperature of the solution is maintained within the range of from about 50°C to about 70°C during the passage of the electric current therethrough.

In accordance with another preferred embodiment of the process of this invention an electric current at a density in the range of from about 5 to about 150 amperes per square foot of electrode surface is passed through an aqueous alkaline solution containing complexes of divalent nickel ions and potassium salts of the EDTMP-HEDP ligands, i.e., hexapotassium ethylenediamine tetra(methylene phosphonate) and tetrapotassium 1-hydroxy, ethylidene-1,1-diphosphonate, having a pH in the range of from about 8.0 to about 10.5. The concentration of the composition containing these complexes in the solution is sufficient to provide from about 1 percent to about 5 percent by weight, based on the weight of solution, of nickel and the temperature of the solution is maintained in the range of from about 50°C to about 70°C during the passage of the electric current therethrough.

It is to be understood that the plating (galvanic) solutions of the present invention can contain the known brighteners, buffers, and leveling agents and other additives. Boric acid and its salts are the compatible buffers for many formulas of the invention. The known brighteners suitable for a certain metal, when present in the galvanic solutions described here, are in general beneficial for the same metal; for example, selenites and arsenites are useful for the copper plating bath and aldehydes and ketones for the zinc plating bath.

Other additives which may be employed in the electroplating solutions of the present invention are disclosed in the 39th Annual Edition, *Metal Finishing*

*Guidebook Directory For 1971*, published by Metals and Plastics Publications, Inc., 99 Kinderkamack Road, Westwood, New Jersey, and which publication is incorporated herein by reference.

The following Examples are intended to illustrate the invention but not to limit the scope thereof, parts and percentages being by weight unless otherwise specified.

#### EXAMPLE I

10 Approximately 22 tests were conducted in this Example in order to show the cooperative effect of the HEDP and EDTMP ligands in the electrodeposition of metals from an electroplating solution containing such ligands, as contrasted to the utilization of these ligands on an individual basis.

20 Twenty two plating solutions were individually prepared in a glass beaker in the following manner. The solutions were prepared in deionized water by first adding potassium hydroxide followed by the particular ligand and then a copper salt which was copper sulfate. Final adjustment of the pH of each solution was made with the addition of potassium hydroxide. The pH of each solution was approximately 8.0. It was noted that considerable heat was evolved during the addition of

25 the ligand to the potassium hydroxide aqueous solution and that the temperature reached 60°-70°C within a few minutes. This temperature range resulted in a quick dissolution of the ligand and the copper sulfate into the aqueous solution. In certain instances, when

30 the copper sulfate would not dissolve at the 60°-70°C temperature range, the solution was heated up to 80°C and stirred vigorously for an additional 20 minutes. The solutions were cooled, if necessary, to the plating temperatures indicated in Table I and transferred from a beaker to a "Hull Cell." The particular ligand utilized, the ligand to copper mol ratio and the percent copper in solution are all shown in Table I.

35

TABLE I

Electroplating of brass and steel cathodes with Cu<sup>++</sup> at pH 8.0 in a 1,000 ml. Hull Cell<sup>1</sup>

| Test No. | Ligand     | Ligand/Cu ratio <sup>2</sup> | Percent Cu in solution <sup>3</sup> | Temp., °C. | Brightness range <sup>4</sup> | Brightness rating <sup>5</sup> | Remarks on brightness quality                   |
|----------|------------|------------------------------|-------------------------------------|------------|-------------------------------|--------------------------------|-------------------------------------------------|
| On brass |            |                              |                                     |            |                               |                                |                                                 |
| 1.       | HEDP       | 1:1                          | 2                                   | 60         | 0-0                           | Poor                           | Smudged, foggy, spotted.                        |
| 2.       | HEDP       | 2:1                          | 2                                   | 60         | 0-68                          | Poor to fair                   | Smudged, foggy, spotted better than Test No. 1. |
| 3.       | HEDP       | 4:1                          | 1                                   | 60         | 0-75                          | Fair                           | Better than Test No. 2.                         |
| 4.       | HEDP       | 4:1                          | 1                                   | 40         | 0-50                          | Poor                           | Dull plate.                                     |
| 5.       | HEDP       | 4:1                          | 1                                   | 70         | 0-75                          | Fair                           | Bright plate but smudged and foggy.             |
| On steel |            |                              |                                     |            |                               |                                |                                                 |
| 6.       | HEDP       | 1:1                          | 2                                   | 60         | 0-0                           | Poor                           | Smudged, foggy, bad adhesion.                   |
| 7.       | HEDP       | 2:1                          | 2                                   | 60         | 0-60                          | Poor to fair                   | Smudged, foggy, very good adhesion.             |
| 8.       | HEDP       | 4:1                          | 1                                   | 40         | 0-60                          | Poor                           | Dull plate, poor adhesion.                      |
| 9.       | HEDP       | 4:1                          | 1                                   | 60         | 0-70                          | do                             | Poor adhesion.                                  |
| On brass |            |                              |                                     |            |                               |                                |                                                 |
| 10.      | HEDP       | 2:1                          | 2                                   | 60         | 0-68                          | Poor to fair                   | Smudged, foggy, spotted.                        |
| 11.      | EDTMP      | 0.5:1                        | 2                                   | 60         | 0-10                          | Poor                           | Bright range too narrow.                        |
| 12.      | EDTMP      | 1:1                          | 2                                   | 60         | 0-28                          | Fair                           | Do.                                             |
| 13.      | HEDP+EDTMP | (1.5+0.5):1                  | 2                                   | 60         | 0-80                          | Good                           | Bright, smudged, foggy.                         |
| 14.      | HEDP+EDTMP | (1.5+0.5):1                  | 2                                   | 70         | 0-150                         | do                             | Do.                                             |
| 15.      | HEDP+EDTMP | (4+0.5):1                    | 1                                   | 60         | 0-60                          | Very good                      | Very bright plate, some smudges.                |
| 16.      | HEDP+EDTMP | (4+0.5):1                    | 1                                   | 70         | 0-150                         | do                             | Very bright plate, some smudges, stains.        |
| 17.      | HEDP+EDTMP | (2+0.25):1                   | 2                                   | 60         | 0-100                         | do                             | Very bright plate, two bright regions.          |
| 18.      | HEDP+EDTMP | (2+0.25):1                   | 2                                   | 70         | 0-150                         | do                             | Do                                              |
| On steel |            |                              |                                     |            |                               |                                |                                                 |
| 19.      | HEDP       | 2:1                          | 2                                   | 60         | 0-60                          | Poor to fair                   | Smudged, foggy, very good adhesion.             |
| 20.      | EDTMP      | 1:1                          | 2                                   | 60         | 0-30                          | Fair                           | Bright range too narrow, good adhesion.         |
| 21.      | HEDP+EDTMP | (4+0.5):1                    | 1                                   | 70         | 0-60                          | Good                           | Bright, some stains, fair adhesion.             |
| 22.      | HEDP+EDTMP | (2+0.25):1                   | 2                                   | 60         | 0-100                         | Very good                      | Two brightness regions, very good adhesion.     |

<sup>1</sup> At 5 amperes for 5 minutes using constant supply of current and agitating the bath by bubbling into it compressed cylinder air.

<sup>2</sup> Molar ratio of Ligand acid, 100%, to Cu<sup>++</sup>.

<sup>3</sup> From CuSO<sub>4</sub>.

<sup>4</sup> The wider the brightness range the better the plating; 0-150 amperes/ft.<sup>2</sup> maximum.

<sup>5</sup> Subjective rating based on the width of the brightness range, uniformity of brightness, good adhesion of Cu to steel, the absence of pronounced smudges, stains and discoloration.

<sup>6</sup> LCDA = low current density area.

The Hull Cell was constructed substantially as the electrolysis cell described in U.S. Pat. No. 2,149,344 (which is incorporated herein by reference) and the galvanic deposition was performed with intermittent agitation. The Hull Cell utilized in this case had a capacity of 1,000 milliliters. This type of Hull Cell is standard equipment for the evaluation of electroplating solutions by the determination of the "brightness range". By subjective evaluation, this permits the formulation of a "brightness rating" which takes into consideration the overall variables utilized in and the end results obtained from the electroplating test. The particular cathodes utilized in this test were brass or steel as so indicated in Table I and were each 5 x 3 1/4 inches in size. The anode utilized in these tests was made of copper and was 2 1/4 x 2 1/4 inches in size.

As noted in the footnotes of Table I, each test was conducted for a period of 5 minutes at a constant current of 5 amperes. The results of these 22 tests are set forth in Table I and particular attention is directed to the column designated "Brightness Rating" which is the basic criteria for an evaluation of the electroplating effects on an overall basis.

Referring to Table I, test Nos. 1 - 5 and 10 were made utilizing the HEDP ligand per se with a brass cathode and the results shown under the brightness rating indicated the overall electroplating effect was "poor to fair". In test Nos. 6 - 9 and 19, utilizing a steel cathode, the brightness rating was also basically poor.

In using the EDTMP ligand in test Nos. 11 and 12, and 20 respectively with brass and steel cathodes, the brightness rating is essentially "poor" in each case.

The unique cooperative effect of the HEDP and EDTMP ligands (i.e., the present invention) is shown in test Nos. 13 - 18, 21 and 22. The cooperative effect of these combined ligands results in a brightness rating ranging from "good to very good." Thus, it can be readily seen that the combination of HEDP and EDTMP results in unexpected results in view of the fact that when either one of these individual ligands is utilized, the results are substantially less than when the two ligands are utilized together.

## EXAMPLE II

The procedure utilized in the above Example I was also utilized in this Example II in order to prepare the solutions and effect the test designated as Nos. 1 - 14 in Table II. Each electroplating solution was adjusted, however, to a pH 10 in this Example II as compared to the pH 8 of Example I plating solutions. The Hull Cell was the same in both examples.

Referring to Table II, test Nos 1 - 4 show the utilization of the HEDP ligand per se with a brass and steel cathode. The brightness ratings of these tests ranged from "fair to good."

Test Nos 5, 6 and 7 show the effect of utilizing the EDTMP ligand per se with brass and steel cathodes. These tests result in brightness ratings of "very bad to poor."

However, when utilizing a combination of the HEDP and EDTMP ligands, test Nos. 8, 9 and 10 result in brightness ratings of "very good" in all three tests with the utilization of both brass and steel cathodes.

Thus the cooperative effect of the HEDP and

TABLE II  
Electroplating of brass and steel cathodes with Cu<sup>++</sup> at pH 10.0 in a 1,000 ml. Hull Cell<sup>1</sup>

| Test No. | Ligand                  | Ligand/Cu ratio <sup>2</sup> | Percent Cu in solution <sup>3</sup> | Temp., °C. | Brightness range <sup>4</sup> , amperes/ft. <sup>2</sup> | Brightness rating <sup>5</sup> | Remarks on brightness quality                   |
|----------|-------------------------|------------------------------|-------------------------------------|------------|----------------------------------------------------------|--------------------------------|-------------------------------------------------|
| On brass |                         |                              |                                     |            |                                                          |                                |                                                 |
| 1.....   | HEDP                    | 2:1                          | 2                                   | 70         | 0-150                                                    | Fair to good.....              | Dark smudges, poor cover in LCDA <sup>6</sup> . |
| 2.....   | HEDP                    | 2.5:1                        | 2                                   | 70         | 0-40                                                     | Fair.....                      | Bright range too narrow.                        |
| On steel |                         |                              |                                     |            |                                                          |                                |                                                 |
| 3.....   | HEDP                    | 2:1                          | 2                                   | 60         | 0-100                                                    | Good.....                      | Bright plate, some smudges, very good adhesion. |
| 4.....   | HEDP                    | 2:1                          | 2                                   | 70         | 0-130                                                    | do.....                        | Very bright plate, fair cover in LCDA.          |
| On brass |                         |                              |                                     |            |                                                          |                                |                                                 |
| 5.....   | EDTMP                   | 0.5:1                        | 2                                   | 60         | 0-10                                                     | Poor.....                      | Brightness range too narrow.                    |
| 6.....   | EDTMP                   | 1:1                          | 2                                   | 60         | 0-0.5                                                    | Very poor.....                 | Very dark plate.                                |
| On steel |                         |                              |                                     |            |                                                          |                                |                                                 |
| 7.....   | EDTMP                   | 1:1                          | 2                                   | 60         | 0-0                                                      | Very bad.....                  | No plating whatsoever.                          |
| On brass |                         |                              |                                     |            |                                                          |                                |                                                 |
| 8.....   | HEDP+EDTMP              | (2+0.25):1                   | 2                                   | 70         | 0-150                                                    | Very good....                  | Very bright, uniform plate.                     |
| On steel |                         |                              |                                     |            |                                                          |                                |                                                 |
| 9.....   | HEDP+EDTMP              | (2+0.25):1                   | 2                                   | 70         | 0-60                                                     | Very good....                  | Very bright, very good adhesion.                |
| 10.....  | HEDP+EDTMP              | (2+0.25):1                   | 2                                   | 70         | 0-75                                                     | do.....                        | Do.                                             |
| On brass |                         |                              |                                     |            |                                                          |                                |                                                 |
| 11.....  | CuCN—Standard (pH 12.0) |                              |                                     |            |                                                          |                                |                                                 |
| 11.....  | CN:Cu                   | 3.8:1                        | 1.22                                | 60         | 0-150                                                    | Good.....                      | Bright plate, dark in the LCDA.                 |
| 12.....  | CN:Cu                   | 3.8:1                        | 2.44                                | 60         | 0-150                                                    | do.....                        | Better than Test No. 11.                        |
| On steel |                         |                              |                                     |            |                                                          |                                |                                                 |
| 13.....  | CN:Cu                   | 3.8:1                        | 1.22                                | 60         | 0-150                                                    | Good.....                      | Bright plate, smudged, very good adhesion.      |
| 14.....  | CN:Cu                   | 3.8:1                        | 2.44                                | 60         | 0-150                                                    | do.....                        | Do.                                             |

<sup>1</sup> At 5 amperes for 5 minutes using constant supply of current and agitating the bath by bubbling into it compressed cylinder air.

<sup>2</sup> Molar ratio of Ligand acid, 100%, to Cu<sup>++</sup>.

<sup>3</sup> From CuSO<sub>4</sub>.

<sup>4</sup> The wider the brightness range the better the plating; 0-150 amperes/ft.<sup>2</sup> maximum.

<sup>5</sup> Subjective rating based on the width of the brightness range, uniformity of brightness, good adhesion of Cu to steel, the absence of pronounced smudges, stains and discoloration.

<sup>6</sup> LCDA=low current density area.

EDTMP ligands in electroplating solutions is vividly illustrated in this Example II as with Example I and show the uniqueness of this combination as compared to the utilization of these ligands on an individual basis.

For a comparative basis, tests 11, 12, 13 and 14 were conducted utilizing copper cyanide as a standard. The brightness rating on all four of these tests was good. This is contrasted to the very good brightness rating with the utilization of the present invention electroplating solutions containing the combination of the HEDP and EDTMP ligands; however, these present invention solutions did not exhibit the disadvantages associated with the copper cyanide solution as heretofore described.

In conjunction with the utilization of the EDTMP ligand per se in an electroplating solution, this usage has been suggested in German Pat. application No. 2,023,304 which was published Nov. 18, 1970 and which publication is incorporated herein by reference. In view of this German publication and the aforementioned U.S. Pat. No. 3,475,293, it can readily be seen that the unique combination of the HEDP and EDTMP ligands of the present invention is an improvement over these publications and is unexpected in view of the results set forth in Examples I and II above.

### EXAMPLE III

Where one so desires to achieve the cooperative effect derived from the present invention, other plating solutions can be prepared and different cathode and anode materials utilized all in an electrodeposition process. Thus, cathodes such as zinc and aluminum can be interexchanged with anodes prepared from copper, nickel, cadmium, iron, zinc, cobalt and cadmiumnickel materials. Furthermore, the plating solutions can be prepared utilizing salts (which supply the metal ion for the HEDP—EDTMP complexes) such as copper carbonate, potassium carbonate, nickel carbonate, cadmium carbonate, iron chloride, zinc oxide, cobalt citrate, sodium zincate, nickel sulfate and iron sulfate.

It is to be understood that the foregoing examples are merely illustrative of the present invention and are not to be considered as restrictive or limiting thereto and that other ramifications can be effected and variables changed all of which are within the scope of the present invention.

What is claimed is:

1. A process for the electrodeposition of a metal which comprises the step of electrolyzing an aqueous solution having a pH of from about 6.0 to about 13.0 of a composition comprising (1) a complex consisting of a metal ion and an ethylenediamine tetra (methylene

phosphonate) ligand and (2) a complex consisting of a metal ion and a 1-hydroxy, ethylidene - 1, 1 - diphosphonate ligand: wherein said composition is present in said solution in an amount sufficient to provide from about 0.1 percent to about 5 percent by weight, based on the weight of said solution, of said metal and wherein said diphosphonate to metal ion mol ratio is from about 1.0:1 to about 4.0:1, and said methylene phosphonate to metal ion mol ratio is from about 0.1:1 to about 1.0:1; said solution being at a temperature in which the solution produces galvanic deposits.

5 2. The process as set forth in claim 1 wherein the metal ion is a transitional metal ion selected from the group consisting of gold, copper, iron, nickel, zinc and cadmium ions.

15 3. The process as set forth in claim 1 wherein such methylene phosphonate ligand is ethylenediamine tetra(methylene phosphonic acid).

20 4. The process as set forth in claim 1 wherein such diphosphonate ligand is 1-hydroxy, ethylidene-1,1-diphosphonic acid.

25 5. The process as set forth in claim 1 wherein said solution is maintained at a temperature of from about 40°C to about 80°C during the electrodeposition of said metal.

30 6. A galvanic bath useful for the preparation of galvanic metal deposits which comprises a substantially cyanide - free aqueous solution having a pH of from about 6.0 to about 13.0 which contains a composition comprising (1) a complex consisting of a metal ion and an ethylenediamine tetra (methylene phosphonate) ligand and (2) a complex consisting of a metal ion and a 1-hydroxy, ethylidene-1, 1-diphosphonate ligand; wherein said composition is present in said solution in an amount sufficient to provide from about 0.1 percent to about 5 percent by weight, based on the weight of said solution, of said metal and wherein said diphosphonate to metal ion mol ratio is from about 1.0:1 to about 4.0:1, and said methylene phosphonate to metal ion mol ratio is from about 0.1:1 to about 1.0:1.

35 7. The bath as set forth in claim 6 wherein said methylene phosphonate ligand is ethylenediamine tetra(methylene phosphonic acid).

40 8. The bath as set forth in claim 6 wherein said diphosphonate ligand is 1-hydroxy, ethylidene-1,1-diphosphonic acid.

45 9. The bath as set forth in claim 6 wherein the metal ion is a transitional metal ion selected from the group consisting of gold, copper, iron, nickel, zinc and cadmium ions.

\* \* \* \* \*